

Dec. 28, 1937.

J. W. HARSCH

2,103,848

## HEAT TREATMENT OF STEELS

Filed May 12, 1934

FIG.2



FIG.3 16b



FIG. I



*INVENTOR.*

BY

INVENTOR  
John H. Harich

Cornelius D. Street  
his ATTORNEY.

## UNITED STATES PATENT OFFICE

2,103,848

## HEAT TREATMENT OF STEELS

John W. Harsch, Gwynedd, Pa., assignor to Leeds  
& Northrup Company, Philadelphia, Pa., a cor-  
poration of Pennsylvania

Application May 12, 1934, Serial No. 725,280

1 Claim. (Cl. 148—16)

My invention relates to methods of heat treating steels or alloy steels.

In accordance with my invention, in the heat-treatment of metals containing carbon, such as 5 steels, alloy steels or the like, decarburization or oxidization, or both, during the heat-treatment are precluded by utilizing as or in an atmosphere, in which the metal is heated, products resulting from cracking of an organic compound, or mixture of organic compounds, comprising carbon, 10 hydrogen and oxygen in fixed or definite proportions.

In accordance with my invention, during heating of articles of hardenable steel to quenching 15 temperature, substantially to prevent loss of carbon at or near the surface of the articles by reaction with such components of the furnace atmosphere as carbon dioxide, water vapor, oxygen, etc., I introduce a hydrocarbon gas or vapor, to 20 provide a component of the furnace atmosphere whose carburizing power is preferably in equilibrium with or slightly greater than the tendency for the articles to lose carbon by reaction with said one or more other components of the furnace 25 atmosphere.

My invention also resides in methods herein-after described and claimed.

Fig. 1 of the drawing illustrates an arrangement for hardening in accordance with my invention;

Fig. 2 shows explanatory curves;

Fig. 3 is a detail view in section and on enlarged scale of parts appearing in Fig. 1.

In general, dies, tools, gears and the like, are 35 hardened by heating them to suitable extent beyond a critical point of the particular steel or alloy of which they are composed, and then quenching them, usually in oil, water or liquid. Heretofore, it has been difficult to avoid defective 40 pieces due to decarburization and formation of scale during the heating period. If the atmosphere in which a work is heated is oxidizing, the surface of the work after being heated to quenching temperature contains less carbon than the 45 core and is too low in carbon content to obtain the desired surface hardness during quenching. The usual result is the formation of soft spots or soft skin on the surface rendering the work unfit 50 for use, or at least shortening its working life. Scale also is formed by oxidizing atmospheres and causes losses because of the difficulty of its removal and the effect upon quenching.

The development of tool and alloy steels requiring 55 high quenching temperatures have accentuated

the difficulties of decarburization and scaling.

Many expedients have been resorted to in attempts to procure a non-oxidizing or neutral atmosphere; for example, combustibles, as oily waste, sawdust, paper and the like have been placed in the furnace to deplete the oxygen; in some cases combusted gases have been used; in oil or gas fired furnaces, the ratio of fuel to air has been controlled to prevent excess of oxygen, 10 etc. Consistent results have not been obtained with any of these methods. Even though the oxygen was exhausted from the heat-treating chamber, the surface of the work was, nevertheless, decarburized to greater or less extent. As a 15 result of investigation, it was found that the decarburization was due to the presence of carbon dioxide, or water vapor, or both. Rapid decarburizing occurred even when the water vapor was as low as .05%. In fact, traces of water vapor 20 from the heat insulating material of the furnace were sufficient to cause decarburization. The furnace atmosphere usually also contains some water vapor, or carbon dioxide, because of infiltration.

Attempts to conserve or replace the surface carbon by dipping the hot pieces in cyanide before quenching, or by covering or packing the pieces with bone black during heating, have not been satisfactory because of the practical impossibility of obtaining consistently good results.

I have found that the effects of water vapor, oxygen, and carbon dioxide, etc., can be offset by heating the work in a slightly carburizing atmosphere; i. e., instead of trying to remove these 35 decarbonizing elements from the heating atmosphere, or subsequently to supply carbon to the work, I add to the atmosphere surrounding the work during heating sufficient carburizing agent 40 to insure that the rate of carburization is equal to or preferably slightly higher than the rate of decarbonization. Theoretically, during the heating, it would suffice to effect equilibrium between the rate at which carbon of the iron is reacting 45 with the decarburizing constituents of the atmosphere and the rate at which carburizing is being effected; but, in practice, the carburizing agent, as a gaseous hydrocarbon, should be supplied slightly in excess, as the resultant formation of a faint soot deposit is visible evidence that the 50 work is in proper condition for quenching; i. e., that the concentration of carbon at or near the surface is the same as, or perhaps slightly higher than the concentration more remote from the 55 surface.

By practice of my method, consistent results are obtained, and actually higher surface hardnesses are produced than were previously obtainable; for example, with oil-quenching steels 4 points (Rockwell "C") increase of hardness has been obtained, and with water-quenching steels an increase of 1½ points has resulted. The surface of the work so heated has no scale, ensuring faster and more uniform quenching action. Improved quenching results are obtained because the surface is kept clean, affording an increased depth of hardening for any given quenching temperature, therefore allowing lower quenching temperatures than before for the same hardness, with consequent less likelihood of distortion.

By way of example, with silverware dies, the production life of dies hardened by my method compared to the production life of dies hardened by prior methods was five or more times longer. Moreover, several hours of stoning were necessary, after hardening by the prior methods, before the dies could be used, whereas, the original finish of the dies, hardened by my method, was restored by a brief light rubbing with crocus cloth. Curves A, C and D, Fig. 2, are hardness curves of three specimens, identical before hardening, and hardened respectively in accordance with my method, and in accordance with the prior method in an electric and a gas furnace whose atmospheres were not controlled. In all three cases the pieces were heated to the same temperature above critical and quenched.

Not only is the surface hardness of specimen A significantly higher than the surface hardness of the other specimens, but its hardness to the center is higher than the greatest hardness of any point of the other specimens, and at the center the hardness of specimen A is tremendously greater than the center hardness of specimens D and C. The superior surface hardness of specimen A resulted from prevention of loss of carbon at and near the surface, and because of rapid quenching action, due to the clean surface of this specimen, the hardness extends far below the surface. Both of the other specimens C and D are of inferior surface hardness due to loss of carbon near the surface; curve C shows this very clearly as the piece at the surface is softer than it is from below the surface to about  $\frac{3}{8}$ " and much softer than at a depth of from about  $\frac{1}{2}$ " to, say,  $\frac{1}{8}$ ". For both specimens C and D, the hardness toward and near the center is poor because the quenching action was impeded by the fouled surface of the pieces.

Moreover, the variation in surface hardness (not shown by Fig. 2) of specimen "A" is only about a half point "Rockwell C", whereas, the surface hardness variation of the others is as much as six times as great.

My method of hardening should not be confused with carburizing in the sense that the term "carburizing" is used in the art. In carburizing, the steels are of low carbon content, e. g., 0.2% or less, and the object is to add carbon to form a high carbon case on the low carbon core. The temperature used in carburizing is chosen to effect penetration into the metal of carbon at a desired rate, and is not functionally related to critical points or temperatures of the steel or corresponding with the decalescent stage; the temperature for carburizing is related only to matter of suitable reaction temperature or the rate of carburization. The work is held at elevated temperature for a long period of time, for example, 75 four hours or usually more. Hardening in gen-

eral, as the term is used in the art, is concerned with straight carbon or alloy steels of high carbon content (about .4 to 1.5% carbon) which are hardened by heating them as rapidly as possible without danger of distortion to a predetermined temperature above their critical or decalescent temperature, and then substantially immediately removing them from the heating chamber and quenching them.

Depending upon the type and capacity of the furnace and the nature and size of the load, the time for hardening may vary considerably, as from a few minutes to perhaps not more than two hours; and, as above stated, the time, in any event, is that required to heat the work to the desired supercritical temperature and is not related to duration of an essential reaction, as in carburizing.

Curves A and B, Fig. 2, illustrate the difference between hardening and carburizing. Curve A represents the hardness curve of a specimen of oil-hardening tool steel hardened in accordance with my method; the steel, before hardening, is of high and uniform carbon content from surface to center, and after hardening, the core, as well as the surface, is hard because of the heat treatment. Curve B represents the hardness curve of a carburized specimen which, before carburization, is of low carbon content and which, after carburizing and hardening, is still of low carbon content (except at and closely adjacent the surface) so that it cannot be materially hardened by heat treatment except at or near the surface.

The inferior sub-surface hardness shown in curve B exists because the core is not capable of being hardened, whereas, the inferior hardness near the center of specimens having curves C and D is due to poor quenching action characteristic of prior hardening methods. As above pointed out, the steel of specimens C and D, if treated in accordance with my method, has the characteristic A, whereas, the specimen of curve B cannot have such a hardness characteristic.

The two processes exemplified by curves A and B are for different types of steels, involve different considerations of time and temperature, and are for obtaining different ends; the steels represented by curves A and B have different fields of use.

In general, my method is contrasted in that it is concerned with the prevention of loss of carbon from the work during heating to a supercritical temperature, and prevention of the surface fouling or formation of scale during that time.

The atmosphere for effecting my method may be prepared by cracking a liquid hydrocarbon in a chamber separate from the hardening chamber. Clean work and freedom from surface decarburization are obtainable by introducing hydrocarbon oils, vapors, or gases into the hardening furnace. However, it was found necessary to take into consideration the fact that a number of equilibrium reactions exist in the furnace between carbon dioxide, carbon monoxide, carbon, water vapor and other breakdown components of the oils. These caused formation of water vapor at certain temperatures and resulted in oxidation and decarburization the effect of which could not always be overcome at the higher temperatures where the equilibrium of the reactions shifted so that water vapor was largely eliminated. Also, the direct introduction of the agent in some types of equipment is apt to cause an excess deposit of

free carbon on the work which, in turn, causes soft spots due to quenching difficulties.

In any event, the supply of carburizing agent should continue during heating, as it has been found that an atmosphere containing hydrocarbon, and carbon monoxide, hydrogen, and/or water vapor decreases in carburizing power with increasing time of exposure in the hardening chamber.

10 It is preferable to use a pre-cracking chamber for preparing the gas or vapor and establishing the desired condition insofar as equilibrium reactions are concerned. The soot, or free carbon, if any, resulting from the cracking, is deposited 15 in the cracking chamber and not in the hardening chamber into which the gas, after preparation, is introduced.

A satisfactory system for performing my method is shown in the drawing, to which reference is now made.

20 A suitable hydrocarbon as ethyleneglycolmono-ethylether, fusel oil or the like, is disposed in a container 1 having a gauge 2 for showing the level. The flow of the liquid through the pipe 3 to the pre-cracking furnace 4 is controlled by a needle valve 5 provided with a sight glass 6. The pre-cracking furnace comprises an inner shell 7 defining a heating chamber and an outer shell 8, the space between which is filled with a suitable 25 heat-insulating material 9. The cylindrical space defined by the inner shell 7 is heated in any suitable manner, preferably by electrical heaters 10, as in the furnace shown in Fig. 1 of Wrighton Patent #1,165,055. Within the shell 7 is disposed the retort 11 having at its upper end a peripheral groove 12 which receives the flange of a removable cover 13. The groove is filled with aluminum oxide or other sealing material to form a sealed cracking chamber. Within the chamber is disposed tube 14 whose lower end opens to the interior of chamber 11 and whose upper end secured to cap 13 and thereby closed with respect to container 11 is in communication with feed pipe 3'. The liquid hydrocarbon falling through pipe 3' which extends through the cover 15 of the furnace, strikes the upper disc 16a of the target assembly 16 within tube 14 which, together with the other structure, is heated to cracking temperatures. The lower disc 16b and the apertured plates 16c, 16d also are part of the 30 target assembly which is supported by a few wires 16e extending across tube 14. The gas formed by the pyrolytic breakdown of the oil passes around the lower end of the tube 14 up around the outer shell 11 to the outlet pipe 17 which extends downwardly through the base 18 of the furnace. The inlet pipe 19 of the hardening furnace 20 which projects through the base 21 thereof into the hardening chamber H is connected to the outlet 17 of the pre-cracker by pipe 22.

#### The cracking of fusel oil



70 ethyleneglycolmonoethylether



75 and like organic compounds of definite composi-

tion comprising hydrogen, carbon and oxygen, for a given cracking temperature results in the production, by reaction endothermic in character, of methane, carbon monoxide, hydrogen and carbon in fixed proportions. The relative proportions of methane and carbon monoxide, the significant components of the furnace atmosphere of definite composition so produced, is controllable by varying the cracking temperature and/or the rate of flow or feed of the fusel oil or equivalent.

10 It has heretofore been proposed in heat-treating methods, such as annealing, to prepare the furnace atmosphere by cracking of various hydrocarbon compounds such as naphtha, mixtures of methane and hydrogen, fuel gas, benzol 15 or tar, but these materials and methods are unsuited to my purposes because, inter alia, these substances or mixtures lack oxygen, either alone or in proper combination, and so fail to provide a carbon-containing atmosphere of proper character.

20 It has also been proposed with substances or mixtures of this latter named character to crack them by a combustion reaction, exothermic in character, by which oxygen, as that of the air 25 or otherwise not present in the substance or mixture, in uncontrollable and widely varying proportions enters into the composition of the resulting products, and in consequence the furnace atmosphere is very indefinite and not suited to 30 my purposes, not only because of the practical impossibility of controlling the amount of oxygen which enters into the reaction, but also because the cracking temperature is the temperature of the reaction itself or dependent upon the reaction and so not to practical extent subject to 35 control or controllable.

40 For quenching temperatures with which my invention is concerned, to wit, ranging from about 1300° F. to about 2000° F., steels or alloy steels of high carbon content are to prohibitive extent decarburized if their heating to proper quenching temperature within the aforesaid range be effected in the presence of an atmosphere consisting of products of combustion, which 45 at higher temperatures, as about 2300° F., do not effect material decarburization.

45 Furthermore, organic compounds of indefinite or inconsistent chemical composition, as tars, bone oil, blast furnace and coke oven gases, are 50 unsuited to my purposes and are not comprehended within my invention, for they do not afford or permit consistently reproducible results because use of them prevents the necessary stability of composition of the furnace atmosphere.

55 Soot and/or tarry deposits resulting from the breakdown of the hydrocarbon fluids, whether gaseous or liquid, are deposited in the pre-cracking unit and are not introduced into the work 60 chamber of the hardening furnace. The construction of the pre-cracking unit, as indicated,

65 is such that it can be readily disassembled for 70 thorough cleaning, which may be necessary at intervals of every day or so. The connecting tubes, such as 17, 19 and 22, may be readily cleaned; for example, by removal of plug 23 of pipe-cross 24, a cleaning rod may be run through 75

the pipe 17. Similarly, removal of plugs 25 and 26 of the pipe crosses 24 and 27 permits the connecting pipe 22 between the units to be freed of any deposits. The target assembly may be removed for cleaning by withdrawing the supporting wires 16e.

The hardening furnace specifically illustrated comprises the inner shell or lining 28 between which and the outer shell 29 is disposed a suitable heat-insulating material 30. The retort which defines the hardening chamber, in which the work is disposed, is heated as by electric resistors 28a, although other sources of heat may be employed, if desired. The top of the furnace 15 is closed by a cover 32 which is provided with an auxiliary cover 33 for the retort, the latter having a flange 34 which is received by the sealing groove 35 of the retort. Aluminum oxide or other sealing material is disposed in the groove to form an air-tight joint. The carburizing gas entering the chamber from pipe 19, flushes out the air and spent gases which are forced out through the pipe 36 which extends through the lid 32. The exhaust gas issuing from pipe 36 is ignited, as by 20 the continuously acting spark-plug S, as a safeguard against asphyxiation.

The metal used for the hardening chamber, the pre-cracking chamber, and the covers thereof, etc., is a nickel chromium alloy such as 25% nickel, 18% chrome, remainder iron, since this material has sufficient resistance to carburization at temperatures within the heat-treating range which is from about 1300° F. to 2000° F. Both the cracking unit and the furnace are fabricated 30 from sheet-metal, rather than made of castings, because of the decreased weight.

The pyrometers 37, 38 permit the temperatures of the pre-cracker and hardening furnace to be determined and controlled, preferably automatically. The temperature of the atmosphere in the hardening furnace will be within the range of from about 1300-2000° F. depending upon the nature of the steel. In general, the temperature within the aforesaid range, is lower for nickel 40 alloy steels and higher for chromium alloy steels. In all cases, the work is heated to a predetermined temperature above the critical point of its steel and then removed for quenching. The atmosphere within the furnace is maintained in a slightly carburizing state by controlling the feed 45 of oil to the pre-cracker.

With the system described, it is possible to heat pieces of work in the hardening chamber to the desired extent above a critical point and, by control 50 of the furnace atmosphere, to maintain a slight carburizing action, loss of carbon from the surface of the work and scaling can be avoided. The furnace temperature and state of the furnace atmosphere being under control, the pieces of successive runs or batches are uniform in character, yielding uniform results upon quenching.

The time at which the work arrives at its critical temperature may be observed by noting the abrupt change or "hump" in the rate of 55 change of the work temperature curve in accordance with the method of Wrighton Patent #1,188,128, which change may be amplified by the arrangement shown in Martin #1,643,582 or, as in Harsch et al. #1,911,191, the determination 60 can be accurately made by observance of the "humps" in a curve indicative of the differences between the work temperature and the furnace temperature existing as the work is being heated, the source of heat being controlled to maintain 65 a constant difference between the work and the

furnace temperature. The "hump" method is not suited for high-speed tool steels, as tungsten-steels, because their critical temperatures are far too low compared to their necessary quenching temperatures; for example, their critical temperatures are about 1600° F., whereas the proper quenching temperatures are about 2300° F.

In general, the work is heated as rapidly as possible without causing distortion to a desired temperature above the critical point during which time the furnace atmosphere is maintained slightly carburizing to prevent loss of carbon from the work, and then the work is removed and quenched. By rapidly stirring or circulating the gas, the concentration of the gas may be maintained highly constant even for dense loads. This can be effected by disposing a fan in the furnace; that is, the hardening furnace may be similar in construction to that disclosed in my application Serial No. 511,694, filed January 28, 1931, 20 Patent No. 2,032,209, February 25, 1936.

It has been found in practice that the rate of quenching is substantially higher than previously obtainable, affording materially greater sub-surface hardness, as shown by curve A, Fig. 2. This is due to the freedom of the surfaces of the pieces from scale, which materially retards the quenching action whether the quenching medium be oil, water, air or other suitable quenching fluid. Because of the higher quenching rate, the quenching temperatures may be lowered, particularly on oil-hardening steel, which is of advantage since it reduces warpage difficulties encountered at higher temperatures.

The rate of heating, the quenching temperature, and the condition of the surface of the work, the three vital factors of hardening, are by my method brought within control so that enhanced surface and subsurface hardness can be obtained consistently.

It is also of advantage to maintain the furnace atmosphere slightly carburizing during heating of previously hardened pieces to suitably high drawing temperature for tempering or toughening, after which the pieces are withdrawn 40 and quenched. Loss of carbon from the surface of the work is prevented, and the surface is kept clean, affording better quenching action. Forcible circulation or agitation of the furnace atmosphere is desirable, as it ensures uniformity 45 of temperature through the load and also ensures that the atmosphere in contact with all parts of the work is slightly carburizing.

I disclaim herefrom the production of the heat-treating atmosphere by cracking naphtha, tar, benzol, fuel gas, or mixtures of methane and hydrogen, and disclaim herefrom methods of heat treatment which involve production of the heat-treating atmosphere by cracking of organic compounds which do not contain oxygen, and methods which involve production of the heat-treating atmosphere by combustion of organic compounds or by cracking them at temperatures of or imposed by combustion.

Nor is there comprehended by my invention any method of hardening, tempering or toughening of steels and alloy steels, of high carbon content, in accordance with which the steel is heated to a quenching temperature in the presence of products of cracking of an organic compound or 60 compounds comprising carbon, oxygen and hydrogen in definite proportions, and the effect of either substantially decarburizing or substantially carburizing the steel and so to have caused material change in the carbon content of the 7

steel at its surface at the time of quenching; or any method in accordance with which products of combustion are utilized for protective atmosphere, which products of combustion, at the temperatures utilized by me, do not in practice prevent material decarburization of high carbon steels which are quenched at temperatures of about or below 2000° F.

What I claim is:

5 10 In the art of hardening, tempering or toughening steels or alloy steels of high carbon content, the method of maintaining, during heating to quenching temperature within a range of from about 1300° F. to 2000° F., the carbon content of

the steel substantially constant and its surface in condition ensuring high rate of and uniform quenching, which comprises bringing the steel to quenching temperature, simultaneously providing about the steel an atmosphere comprising products of endothermic cracking of an organic compound, or mixture of organic compounds, of chemically definite composition of carbon, hydrogen and oxygen, and maintaining in said atmosphere a concentration of carbon preventive of 5 10 oxidation and decarburization of and case-formation upon the steel.

JOHN W. HARSCH.